

Oct. 16, 1928.

1,688,300

G. D. WELTY

PROCESS OF MAKING HOLLOW ARTICLES

Filed Aug. 2, 1924



INVENTOR

George Donald Welty  
BY  
Rickey, Slough & Welty  
ATTORNEY

## UNITED STATES PATENT OFFICE.

GEORGE DONALD WEILY, OF CLEVELAND, OHIO, ASSIGNEE TO ALUMINUM COMPANY OF AMERICA, OF PITTSBURGH, PENNSYLVANIA, A CORPORATION OF PENNSYLVANIA.

## PROCESS OF MAKING HOLLOW ARTICLES.

Application filed August 2, 1924. Serial No. 729,683.

This invention relates to annular metallic articles, particularly expanded or contracted tubular articles and to a method of making such articles.

5 It further relates to a method of making tubular articles which are to be split in a longitudinal direction by which the tendency of the article to expand or contract when split, as well as the amount of such expansion or 10 contraction, may be determined and controlled.

It also relates to a method of making an annular metallic article adapted to expand or contract radially a predetermined and 15 controllable amount when split lengthwise.

It further relates to a tubular article characterized by possessing increased resistance to contraction or collapse when split lengthwise for a part or all of its length.

20 My invention is based on the discovery that internal strains of compression or tension may be put into a tubular, metallic article by cooling the outside and inside at different rates and that these strains may be predetermined and controlled so that when the wall of the 25 article is split in a longitudinal direction throughout all or part of its length, it will tend to expand or to contract according to the nature and the magnitude of the strains 30 which have been set up.

The preferred method of practicing my invention consists briefly of suitably quenching or cooling the exterior or interior of a suitably heated annular or tubular article at 35 an unequal rate to set up internal strains of tension or compression of the desired magnitude, then splitting the article in a lengthwise direction, the determination of the surface to be cooled the more rapidly depending on whether expansion or contraction of the article, after splitting, is desired.

In the drawings accompanying this specification and forming a part thereof, in which I have illustrated two different structures embodying my invention.

Figure 1 is a perspective view of a tubular article upon which my invention may be practiced.

Figure 2 is a cross sectional view taken on line 2—2 of Fig. 1 showing a tube subjected to my improved process before and after being split lengthwise.

Figure 3 is a view corresponding to Fig. 2

but showing, before and after splitting, a tube subjected to the variation of my process 55 to cause contraction after splitting.

Figure 4 is a cross sectional view of a conventional form of piston provided with circumferentially and longitudinally extending intersecting slits in the skirt, and 60

Figure 5 is a cross sectional view taken substantially on line 5—5 of Fig. 4 showing before and after splitting the piston of Fig. 4 which had been subjected to my method to produce expansion or splitting. 65

Annular metallic articles when suddenly cooled or quenched from fairly high temperatures have internal strains set up in them which strains depend on the nature and extent of the chilling. If the rate of chilling is unequal on the inner and outer surfaces of the article, the strains tend to distort the article when it is split lengthwise, the distortion occurring in a direction dependent upon the place of application of the greater chilling 70 action and to an amount dependent upon the extent of the chilling action. For example, an annular or tubular article may be quenched in a manner to cause the article, when split lengthwise, to contract or to expand, or to remain unchanged; and by suitably regulating the extent of the quenching of the article, the amount of this contraction or expansion 75 may be predetermined and repeated with a high degree of uniformity. 80

My invention is broadly applicable to metallic articles which are, in general, annular, tubular or continuous hollow shells and it is not restricted to such articles when composed of any particular metal or alloy. It may be practiced on cast articles or those which have been previously worked. For example, my method of treatment may be practiced on drawn or extruded tubes of steel, aluminum alloys or other metals, as well as on pistons 90 for internal combustion engines, composed of cast iron or aluminum base alloys. It will, of course be understood that articles of various shapes, sizes and compositions will require different quenching temperatures and 100 that the determination of such temperatures will depend upon the composition and nature of the article in question, and the amount of distortion desired in the treated article. In general the strains are proportional to the 105 severity of the chilling consequently sub-

stantially the same amount of distortion may be obtained by quenching from different temperatures provided the quenching agent or the temperature thereof is suitably varied to 5 cause substantially the same rate of cooling. For example, an article may be cooled from a high temperature by a relatively slow cooling medium and a similar article may be given substantially the same properties by cooling 10 from a lower temperature with a more rapid cooling agent. The specific examples given hereinafter will serve, however, to guide those skilled in the art in practicing my invention on articles of various sizes, shapes, natures 15 and compositions.

In the drawings—Figs. 1, 2 and 3 are various views of a drawn steel tube 1. This tube, when heated to about 1500° F. and then cooled by quenching the inner surface, will 20 possess the property of expanding from the dotted line position to the full line position of Fig. 2 when it is split lengthwise as by slit 2. After being split, the tube 1 may still retain the property of further expansion when 25 it is heated sufficiently or when it is struck or jarred so as to relieve the internal strains. If the outer surface instead of the inner surface is quenched from a temperature of about 1500°, the tube will then possess the property 30 of contracting upon being slit lengthwise, as shown in Fig. 3 where the dotted lines indicate the position of the tube before splitting and the full lines the position after splitting. It will be understood that these indicated 35 changes are greatly exaggerated in the figures, the actual change being only a few thousandths of an inch. With a three inch tube having walls  $\frac{1}{16}$ " thick the expansion or contraction may amount to between about 40 .001" and .003" when quenched from 1500° F. in water at a temperature of about 50° F.

In general, the more severe the quenching the greater will be the tendency of the article to expand or contract, that is, distort and 45 when the quenching of a number of similar articles is of substantially the same severity, the articles will possess the tendency of distortion to substantially the same extent.

My invention is of particular utility when 50 applied to an internal combustion engine piston of the so-called "split skirt" type, wherein one or more of the bearing faces of the skirt are provided with intersecting circumferential and longitudinal slits. In pistons 55 of this type treated in accordance with this invention there is a tendency toward expansion of the free ends of the sections in the skirt along the lengthwise slit, as contrasted with a corresponding tendency to contraction, 60 or to contraction of one section and expansion of another section in permanent mold cast pistons not so treated. Equal expansion of these split sections is desired because it tends to maintain undiminished the original bearing 65 area of the skirt and to make possible

close fitting of the piston to its cylinder and maintenance of substantially the original clearance during the major part of or all the life of a piston.

In applying my invention to tubular articles having a closed end, as illustrated by an internal combustion engine piston, distortion may be produced in the same manner as in the tube shown in Figs. 1 to 3, inclusive, except that in the piston the actual distortion may 70 be confined to a portion only of the skirt, whereas in Figs. 1, 2 and 3 it has been illustrated as being more or less uniformly distributed throughout the entire circumferential length of the article.

Figs. 4 and 5 show a conventional form of piston 3 having a circumferentially extending slit 4 and a longitudinally extending slit 5 intersecting therewith, these slits being formed in what is known as one of the two bearing faces 6 of the piston. The dotted and full lines in Fig. 5 indicate respectively, the 80 positions before and after slitting of a piston skirt subjected to my method to cause expansion after splitting, the amount of change being greatly exaggerated. The piston 3, when cast in a permanent mold of an aluminum base alloy containing say between about 4% and about 16% of copper or copper and 85 other heat responsive hardening metals, such as silicon and magnesium, with or without nickel, manganese, chromium, and with or without other metals, may be subjected to my improved process in one or more different 90 ways.

It may be suitably quenched or may be cooled more rapidly on the inner than on the outer surface, as it comes from the mold in a highly heated condition, and then split; or it may be cooled in the open air to room temperature after being removed from the mold 100 then reheated at a high temperature for the desired length of time, quenched more rapidly on the inner than on the outer surface and then split; but preferably it should be cooled in the open air to room temperature after 105 leaving the mold, then heated to a high temperature for the desired length of time, quenched more rapidly on the inner than on the outer surface, then aged at a low temperature 110 as compared with the high temperature just mentioned, in order to improve such properties as hardness and elastic limit, then machined and split just before putting into the motor. The unequal cooling or quenching step of my method may be accomplished 115 by bringing water, oil or other cooling fluid into the interior thereof, after which the skirt may be split substantially, as shown in Figs. 4 and 5, with the result that the portions of the skirt adjacent to the slits 4 and 5 will 120 tend to assume substantially the full line positions shown in Fig. 5.

When a diametrical expansion of from 125 about .001" or .005" is desired in the skirt 130

of a piston about 3 inches in diameter and composed of an aluminum base alloy of the foregoing composition, I may quench the interior of the piston from temperatures of 5 700° F. to 950° F. but to produce the same result at the lower temperature the temperature of the quenching medium should be correspondingly lower so as to produce the same severity of chilling.

10 The preferred temperature is 950° F. with such compositions because at such temperature the article possesses the maximum potentiality for hardening.

15 The temperature of the quenching medium such as water, to be used with a piston of the foregoing composition and at 950° F. is about 50° F. when an expansion of from .001" to about .005" is desired. Although water has been mentioned hereinabove as a 20 suitable quenching medium, it will be understood by those skilled in the art that oil may be similarly employed, but when the same severity of chill is desired the temperature of the oil should be considerably lower 25 than that of the water. For example, when the cast iron tube mentioned hereinabove is to be quenched from a temperature of about 1500° in oil instead of water, the oil should be maintained at somewhere about 30° F. in 30 order to obtain the same severity of chill as when the water is employed at a temperature of about 50° F.

35 Pistons of such composition when quenched in accordance with my invention not only expand when split but possess the property of tending to expand still more when struck, jarred or subjected to the ordinary usage of pistons in internal combustion engines. They are thus capable of resisting any tendency 40 of the skirt portions along the slits to spring inwardly when the skirt is split or to be pressed inwardly by the cylinder walls.

45 When the inner and outer surfaces of an article heated in accordance with my invention are quickly cooled or quenched at substantially the same rate, the internal strains are either absent or tend to balance each other and the article tends neither to expand nor contract when split lengthwise thereafter.

50 I believe the strains set up by my treatment to be strains of compression and tension; and that in general when one surface of an annular article is quenched by my method that surface has compression strains set up in it while the opposite surface has tension strains set up in it. This belief and theory may not be the real explanation, however, and consequently I do not wish to be bound thereby. The scope of my invention is set forth in what is claimed.

55 What is claimed is:

1. The method of making an annular metallic article which comprises subjecting the

inner and outer surfaces of a circumferentially continuous annular metallic article in a mechanically unrestrained condition respectively to heat treatments differing in degree thereby setting up internal compression 70 strains near one surface in excess of similar strains near the other surface, and then slitting the article in a lengthwise direction for at least a part of its length.

2. The method of making an annular metallic article having a longitudinally extended slit which comprises heating a circumferentially continuous annular metallic article in a mechanically unrestrained condition, to such a temperature that sudden and unequal 75 cooling or quenching of the surfaces will set up unbalanced strains therein, quenching one surface of the said article in a manner to set up greater strains adjacent thereto than adjacent to the other surface, and splitting the 80 article lengthwise for a part or all of its length.

3. The method of making an expanded annular metallic article which comprises heating a circumferentially continuous annular metallic article in a mechanically unrestrained condition to such a temperature that internal 85 strains will be set up therein when the surfaces of the article are suddenly and unequally cooled or quenched, quenching the inner 90 surface of the article in a manner to set up greater strains adjacent thereto than adjacent to the outer surface, and splitting the 95 article lengthwise for a part or all of its length.

4. The method of making an annular, metallic article which comprises subjecting the inner and outer surfaces of a circumferentially continuous annular metallic article in a mechanically unrestrained condition respectively to heat treatments differing in degree thereby setting up internal unbalanced 105 strains in the said article, and then splitting the article in a lengthwise direction for at least a part of its length.

5. The method of making a contracted annular metallic article which comprises heating a circumferentially continuous annular metallic article in a mechanically unrestrained condition to such a temperature that internal strains will be set up therein when the surfaces of the article are suddenly and unequally cooled or quenched from the said 110 temperature, quenching the outer surface of the said article from the said temperature in a manner to set up the internal strains of greatest magnitude adjacent to the inner surface thereof, and splitting the article in a lengthwise direction for a part or all of its 115 length.

6. The method of making an expanded tubular article composed of an aluminum base alloy, which comprises heating an unsplit tubular article composed of such material to a temperature of between about 700° F. 120

to 950° F., quenching the inner surface thereof in a manner to set up the internal strains of greatest magnitude adjacent to the inner surface, and then splitting the said article 5 lengthwise for at least a part of its length.

7. The method of making a contracted tubular article composed of an aluminum base alloy, which comprises heating an unsplit tubular article composed of such material to 10 a temperature of about 950° F., quenching the outer surface thereof in a manner to set up the internal strains of greatest magnitude adjacent to the outer surface and then splitting the said article lengthwise for at least 15 a part of its length.

8. The method of providing an internal combustion engine piston with an expanded skirt which comprises acting upon the circumferentially continuous skirt of a piston 20 in a manner to set up interior compression strains in the inner surface of the skirt portion of the piston, and then forming intersecting slits in the said skirt.

9. The method of providing an internal 25 combustion engine piston with an expanded skirt which comprises heating a piston having a circumferentially continuous skirt portion to such a temperature that interior compression strains will be set up near the surface 30 of the skirt when the surface thereof is suddenly cooled or quenched, quenching the inner surface of the said skirt, and forming intersecting slits in the skirt portion of the said piston.

10. The method of providing an interior 35 combustion engine piston with an expanded skirt and composed of an aluminum base alloy which comprises heating a piston having a circumferentially continuous skirt and composed of an aluminum base alloy to a temperature from about 700° F. to about 950° F., quenching the interior surface of the said skirt and finally forming intersecting slits in the said skirt. 40

11. The method of providing an internal 45 combustion engine piston composed of an aluminum base alloy with an expanded skirt which comprises heating an aluminum base alloy piston casting having a circumferentially continuous skirt to a temperature of 50 between about 700° F. to about 950° F., cooling the heated casting in a manner to set up internal compression strains near the inner surface thereof, and forming intersecting slits in the skirt of the cooled casting. 55

12. The method of providing an aluminum 60 base alloy piston with a skirt of the split type which comprises heating a piston having a circumferentially continuous skirt to a temperature of approximately 950° F., cooling the piston by quenching the inner surface of the skirt in oil or water and forming intersecting slits in the skirt of the thus cooled piston. 65

In testimony whereof I hereunto affix my signature this 29th day of July, 1924.

GEORGE DONALD WELTY.